

April 18, 1933.

F. RINGER

1,903,838

IGNITIBLE STICK

Filed April 26, 1929



INVENTOR  
**FERDINAND RINGER**  
*by his attorneys*

*Houeon and Houeon*

## UNITED STATES PATENT OFFICE

FERDINAND RINGER, OF VIENNA, AUSTRIA

## IGNITIBLE STICK

Application filed April 26, 1929, Serial No. 358,383, and in Austria May 5, 1928.

This invention relates to an ignitable stick and a method for making such sticks.

Up-to-date fire making devices comprise, on the one hand, various kinds of mechanical devices such as the well known pocket type of cigar and cigarette lighters, on the other hand, the well known "matches" are used. The former have the advantage that they can be repeatedly used, but the purchasing price is relatively high and the construction is rather complicated and some of their elements must be repaired often. The operation of these mechanical lighters is not simple and in many types the combustible must be renewed from time to time. Matches are by far preferred owing to their simple manipulation. However, they can be used but once and the burnt match forms a troublesome waste product. The demand for a reliable instrument for repeatedly producing fire has not yet been satisfied.

The object of the present invention is to provide an ignitable stick for repeatedly producing fire, combining the simple and handy manipulation of a match with the advantage of repeated use of mechanical cigar lighters. The stick forming the object of the invention may be ignited by rubbing it on a suitable surface just as a common match, and may be blown out by a person's breath and then be ignited anew after the flame has been extinguished. The stick may be manufactured so as to ignite either on any rough surface or only on phosphureted surfaces.

Prior attempts to make matches or lighters capable of repeated ignition have failed because they burned too rapidly or were so explosive that special quenching devices were needed. These quenching devices failed to change their dangerous character or make the prior devices practical.

The match according to the present invention has for its principal component a combustible ground mass which is slow burning and leaves no noteworthy ashy residue. With this ground mass an igniting mass, for example potassium chlorate and sulphur is used in such amounts that after the match is ignited it may be extinguished by simply blowing upon it. When molded, the combustion

velocity of the ground mass is lower than that of weakly nitrated cellulose. This object may be attained for example by using in the ground mass acetyl cellulose. This substance burns more slowly than weakly nitrated cellulose. With this substance are mixed regulating materials such as ammonium oxalate which further retard the speed of combustion since they contain nitrogen or the like and develop combustion hindering cleavage products. The whole mass of the stick has a sufficient stability to permit of striking on ignition surfaces; but the required hardness is not effected by inorganic fillings, but by selecting the ground mass and, if required, by organic hardening substances, as the fillings used in connection with the ordinary ignitable mass of matches on combustion leave behind a considerable residue whereby the repeated ignition would be impaired or entirely prevented. The ignitable stick, according to the present invention, should preferably leave behind no ashes of this kind which, for instance, would envelope the end of the stick like enamel and would have to be removed before the next ignition. Slight ashes, if any, should be voluminous so as to be easily removable by blowing off.

As to its composition the ignitable stick consists of a combustible ground mass (the main constituent) an initial igniter such as oxygen developing substances together with reducing agents and finally substances required for molding the mass, and if desired further substances for retarding the combustion.

Nitrated cellulose, its derivatives, or other substances having similar qualities such as acetyl cellulose, have proved to be especially adapted for the ground mass. There may be added to these ingredients materials to regulate the rate of combustion, the specific quantity to be added being limited so as to give the mass the desired mechanical properties and moldability. Examples of such materials are ammonium oxalate, camphor, naphthalene, nitronaphthalene, naphthyl acetate, phenyl, cresyl, or naphthyl phosphates or carbonates, halides of aromatic hydrocarbons,

acetin, tetramine of hexamethylene etc. either alone or mixed. As oxygen developing substances all known substances of this kind may be taken into consideration, such as potassium chlorate, nitrate, bichromate, minium, lead peroxide, lead nitrate, calcium plumbate and the like. Furthermore a number of the combustibles in common use for making ignitable masses may be employed such as sulphur, antimony sulfide, lead thiosulfate. Furthermore for increasing the frictional sensitivity, small quantities of substances such as glass powder, pumice-stone, kieselguhr, quartz meal may be incorporated into the mass. If desired, inorganic filling substances or coloring matters may be added to a moderate extent. Moreover hardening substances, such as formaldehyde condensation products may be added.

#### 20 Examples

(1) A mass made according to the present invention and easily ignitable on so called phosphorus friction surfaces may be composed as follows: 60-65 parts of nitrocellulose, 6-14 parts of camphor, 11-20 parts of potassium chlorate, about 2.5 parts of potassium bichromate, about 2.5 parts of sulphur, about 2 parts of ammonium oxalate, 5-15 parts of glass powder and 3-10 parts of zinc white.

(2) Nitrocellulose about 15%, acetyl cellulose about 33%, camphor about 3%, sulphur about 6%, potassium chlorate about 22%, tetramine of hexamethylene about 7%, ammonium oxalate about 4%, powdered glass about 10%.

(3) In Example 2, further quantities of acetyl cellulose may be substituted for nitrocellulose and further quantities of tetramine of hexamethylene may be substituted for camphor.

The ignitable sticks made according to the present invention may be manufactured in different ways, for instance, in accordance with the methods of celluloid manufacture. The different additions may be stirred into a concentrated nitrocellulose solution and the mixture poured into molds and the solvent evaporated. Care should be taken to avoid the formation of pores which would impair the uniform combustion of the stick. Otherwise the combustion controlling ingredients may be incorporated into the ground mass by kneading, and the mixture may be expanded to plates by calendering and the plates then cut into suitable pieces. Or a mixture of the components may be prepared and extruded through a mouth piece of suitable form so as to obtain bars or rods which then are cut into sticks, or the mixture may be molded in presses.

Preferably the ignitable sticks according to the invention are inserted into metallic sleeves, provided with a feeding device,

similar to those used in pencils with adjustable lead, from which sleeve the sticks project but little. After the projecting part is burnt off or before the stick is reused or after repeated use the unconsumed stick is pushed forward to the desired length. In this way, by excluding the lateral access of air, the combustion of the stick beyond a predetermined length is prevented. The closing cap of the sleeves may be provided with a friction surface.

The drawing shows a constructional example of the stick according to the invention in longitudinal section.

In the drawing, 1 shows an ignitable stick as described above, 2 shows the metallic sleeve, 3 is a base plate with arms 4 projecting through slots on opposite sides of the metallic sleeve, by means of which arms the base plate and thereby the stick can be pushed forward to any desired length. 6 shows the closing cap of the sleeve, 5 the friction surface on the closing cap.

The ignitable sticks may also be used in cigar lighters and similar devices where they would form an advantageous substitute for the usual mechanically operated cigar lighter. If so used their combustion velocity and consequently also the composition may vary within wide limits. Furthermore the ignitable stick may also be used as a substitute for solidified alcohol in which case the addition of potassium chlorate may be reduced or entirely dispensed with.

In my copending application Serial No. 430,382, filed February 21st, 1930, I have disclosed and claimed broadly a composition for a purpose similar to the purpose of the invention disclosed herein.

Having described my invention what I claim and desire to secure by Letters Patent is:

1. A combustible composition which when made in stick form may be blown out with a person's breath and then relighted by friction, comprising in the approximate proportions stated, 15% nitrocellulose, 33% acetyl cellulose, 3% camphor, 6% sulphur, 22% potassium chlorate, 7% hexamethylenetetramine, 4% ammonium oxalate, 10% powdered glass.

2. A combustible composition which when made in stick form may be blown out with a person's breath and then relighted by friction, comprising in the approximate proportions stated, a base mass of the class consisting of nitrocellulose, acetyl cellulose and mixtures of these 48%, a friction substance 10%, an oxygen carrier 22%, a combustible substance sensitive to friction, 6%, substances for retarding combustion and improving moldability 14%.

3. A combustible composition which when made in stick form may be blown out with a person's breath and then relighted by friction

tion, comprising in the approximate proportions stated, a base mass of the class consisting of nitrocellulose, acetyl cellulose and mixtures of these 48%, a mixture for improving moldability 10%, a substance for retarding combustion 4%, an oxygen carrier 22%, a substance sensitive to friction 7%, a friction substance 10%.

4. A combustible composition which when made in stick form may be blown out with a person's breath and then relighted by friction, comprising in the approximate proportions stated, a base mass comprising nitrocellulose and acetyl cellulose 48%, a combustion retarding mixture comprising camphor and hexamethylenetetramine and ammonium oxalate 14%, an oxygen carrier 22%, a combustible substance sensitive to friction 6%, a friction substance 10%.

5. A combustible composition which when made in stick form may be blown out with a person's breath and then relighted by friction, comprising in the approximate proportions stated, a base mass of the class consisting of nitrocellulose, acetyl cellulose and mixtures of these in the neighborhood of one half of the total composition, oxygen carriers in the neighborhood of one fifth of the total composition, friction substances in the neighborhood of one tenth of the total composition, substances reducing the rate of combustion and improving moldability, in the neighborhood of one seventh of the total composition, a substance sensitive to friction, one sixteenth or less of the total composition.

6. A combustible composition which when made in stick form may be blown out with a person's breath and then relighted by friction, comprising in the approximate proportions stated, 60-65 parts of nitrocellulose, 6-14 parts of camphor, 11-20 parts of potassium chlorate, 2.5 parts of potassium bromate, 2.5 parts of sulphur, 2 parts ammonium oxalate, 5-15 parts glass powder, and 3-10 parts of zinc white.

7. A combustible composition which when made in stick form may be blown out with a person's breath and then relighted by friction, comprising in the approximate proportions stated, a base mass of the class consisting of nitrocellulose, acetyl cellulose and mixtures of these, 60-65 parts, oxygen carrier 11-22.5 parts, substance sensitive to friction 2.5 parts, friction materials 5-15 parts, substances to reduce the rate of combustion and to improve moldability 6-16 parts.

8. A combustible composition which when made in a stick may be blown out by a person's breath and relighted by friction comprising, in approximately the proportions stated, a base mass of nitrocellulose and acetyl cellulose 48%, substance sensitive to friction and an oxygen carrier 28%, hexamethylene tetramene 7-10%, combustion retarding and friction substances 14%.

9. A combustible composition which when made in a stick may be blown out by a person's breath and relighted by friction comprising, in the approximate proportions stated, acetyl cellulose up to 48%, an oxygen carrier and a substance sensitive to friction 28%, substances for improving moldability 7-10%, a substance to retard combustion 4% and a friction substance 10%.

In testimony whereof I have affixed my signature.

FERDINAND RINGER.

80

85

90

95

100

105

110

115

120

125

130